

Aug. 25, 1953

D. L. EASTMAN  
SCOURING IMPLEMENT  
Filed Aug. 3, 1950

2,650,158



FIG. 1



FIG. 2

INVENTOR.  
DON L. EASTMAN  
Bk  
*W. Foley*  
ATTORNEY

Patented Aug. 25, 1953

2,650,158

# UNITED STATES PATENT OFFICE

2,650,158

## SCOURING IMPLEMENT

Don L. Eastman, Watertown, N. Y., assignor to  
The Carborundum Company, Niagara Falls,  
N. Y., a corporation of Delaware

Application August 3, 1950, Serial No. 177,472

4 Claims. (Cl. 51—298)

1

This invention relates to abrading articles and particularly to scouring implements suitable for general household scouring and cleansing purposes such as the scouring and cleaning of pots and pans and other utensils and equipment in the kitchen and also for the cleaning of porcelain bathroom equipment, painted and enameled woodwork and the like.

This application is a continuation-in-part of my application Serial No. 111,547, filed August 20, 1949, and now abandoned, which in turn is a continuation-in-part of my former application Serial No. 725,361, filed January 30, 1947, now abandoned.

The scouring implement of the present invention is composed throughout of materials which are resistant to deterioration by hot water up to at least 180° F., soap, detergents, solutions of acids and alkali, oils, fats and greases, etc., such as are found in dishwater, and features a pad or supporting layer of elastic, compressible, flexible and pliable material provided with a surface layer of comminuted abrasive material embedded in an adhesive which adhesively secures the abrasive layer to the backing pad, the adhesive layer being comparable to the backing in permanent elasticity, flexibility and pliability so as not to detract in any way from those desirable properties of the backing or base layer, and being also capable of resisting deterioration by hot water, soaps, detergents and the like.

Many materials and devices have been heretofore proposed for various household cleansing and scouring purposes but each one has had certain undesirable features. One common device which has received widespread use as a kitchen scouring material has been a small pad of steel wool or other stranded metal wire or ribbon filaments, which, however, has the disadvantage of breaking down in use with discomfort to the user. Loose abrasive powders have also been employed for cleansing purposes but such materials are unsatisfactory by reason of their tendency to combine with the greases and detritus so that when the resulting mass is washed down the sink or drain it becomes lodged in the drainage lines and builds up solids, caked deposits which ultimately seriously interfere with the proper drainage and eventually clog the drainage line.

Attempts which have heretofore been made to load various plastic or elastic bodies with various abrasive materials, as far as is known, for one reason or another have been unsatisfactory and have met with little or no success.

It is an object of the present invention to pro-

vide an improved scouring implement which avoids many of the disadvantages of the materials heretofore offered for such use.

The abrasive article or scouring implement of this invention differs from articles heretofore used in that the entire article, including the base or supporting layer and the superposed adhesive layer containing abrasive material, is elastic, flexible, compressible, and pliable, and also resistant to deterioration by hot water, soap, detergents, and the acids, alkalies, etc. commonly found in dishwater.

In accordance with the present invention an improved scouring and cleansing implement is constructed of a layer of foam rubber to which a thin surface layer of granular abrasive material is adhesively secured by means of a water-insoluble adhesive, the entire article being substantially unaffected by and non-reactive with the commonly used household soaps and detergents. The foam rubber backing of the present implement can be of any desired thickness but it is preferred to use a layer of foam rubber in the neighborhood of  $\frac{1}{4}$  to  $\frac{1}{2}$ " in thickness as being the most convenient to handle in various manual household usage. The adhesive which secures the abrasive particles to the foam rubber backing is not only water-insoluble and resistant to soaps and detergents, and household fats and greases and other substances commonly found in dishwater, but also has a permanent flexibility and elongation after it has been applied to the foam rubber backing and set to a non-tacky condition. The adhesive is also strongly adherent to both the foam rubber backing and the particulate abrasive material. I have found that blended rubber-resin compounded adhesives composed of a natural or synthetic rubber base blended with a resin such as a phenol-aldehyde resinous condensation product together with suitable compounding ingredients which are conventional and well-known in the art of rubber based adhesives are highly satisfactory for the purpose.

In order that the present invention may be more clearly understood, reference is made to the drawings, in which,

Figure 1 is a perspective view of a scouring pad suitable for household scouring and cleansing purposes and made in accordance with the present invention; and

Figure 2 is a vertical sectional view through the line 2—2 of Figure 1.

The scouring pad shown in the drawing consists of a backing layer 4 of foam rubber about  $\frac{1}{2}$ " in thickness to which a layer 5 of granular

## 3

abrasive material is adhesively secured by means of a layer of adhesive binder 6.

The described abrasive pad can be made as follows:

A layer of foam rubber  $\frac{1}{2}$ " in thickness is first given a primer coat of an adhesive composition such as one of those hereinabove set forth and dried for 2 to 5 minutes at 220° F. The side of the foam rubber which has received the prime coating of adhesive is then given a further coating of adhesive known as the making coat. While the making coat of adhesive is still tacky a layer of granular abrasive of the desired grit size, as for example a layer of 36 mesh grit size granular fused aluminum oxide, is deposited on the adhesively coated surface and a final sizing coat of adhesive applied over the top of the abrasive-coated surface. The coated product is then dried for 2 to 5 minutes at 220° F. followed by a final drying period of 30 minutes at 240° F. to set the adhesive to a non-tacky condition. The adhesive may be applied by roll coating, dip coating or spraying as may be desired. A thin film of adhesive can be applied, if desired, to the reverse side of the foam rubber pad to give it additional strength and wearing qualities.

The granular abrasive used in making scouring pads of the present invention, although specified above as being fused aluminum oxide particles of 36 grit size, can be any of those natural or artificially made mineral abrasive materials available on the market such as emery, various grades of fused aluminum oxide, silicon carbide, silica, garnet or the like and can be of any desired particle size.

The following are typical rubber-resin blended adhesive compositions which have been prepared and used with satisfactory results in the making of abrasive scouring implements in accordance with the present invention:

## No. 1 formulation

|                           | Parts |
|---------------------------|-------|
| Polychloroprene           | 900   |
| Magnesium oxide           | 90    |
| Wood rosin (Type FF)      | 45    |
| Zinc oxide                | 45    |
| Phenyl-beta-naphthylamine | 9     |
| Benzene                   | 1690  |
| Trichloroethylene         | 2850  |
| Sulfur                    | 27    |
| Aniline-butyraldehyde     | 12    |

## No. 2 formulation

|                                                                     | Parts |
|---------------------------------------------------------------------|-------|
| Butadiene-acrylic nitrile copolymer                                 | 100   |
| Durez Resin 12686                                                   | 75    |
| Sulfur                                                              | 3     |
| Phenyl-beta-naphthylamine                                           | 1     |
| Mercaptobenzothiazole                                               | 60    |
| Zinc oxide                                                          | 5     |
| Liquid (refined coal tar oil fraction) plasticizer (such as Bardol) | 10    |

## No. 3 formulation

|                                                                     | Parts |
|---------------------------------------------------------------------|-------|
| Butadiene-acrylic nitrile copolymer                                 | 100   |
| Bakelite Resin BR-17867                                             | 30    |
| Sulfur                                                              | 3     |
| Phenyl-beta-naphthylamine                                           | 70    |
| Mercaptobenzothiazole                                               | 1     |
| Zinc oxide                                                          | 5     |
| Liquid (refined coal tar oil fraction) plasticizer (such as Bardol) | 5     |

## 4

## No. 4 formulation

|                                      | Parts |
|--------------------------------------|-------|
| Polychloroprene                      | 100   |
| Extra light calcined magnesium oxide | 5     |
| Sulfur                               | 0.5   |
| Benzothiazyl disulfide               | 1     |
| Phenyl-beta-naphthylamine            | 1     |
| Rosin                                | 5     |
| Bakelite Resin BR-17867              | 10    |

10 Durez Resin No. 12686, referred to in the above formulation No. 2, is an A stage, phenol-formaldehyde resin in lump form sold by the Durez Plastics and Chemicals, Inc. of North Tonawanda, New York.

15 Bakelite Resin BR-17867, referred to in formulations Nos. 3 and 4 above, is a liquid A stage, phenol-formaldehyde resinous condensation product sold by the Bakelite Corporation of Bloomfield, New Jersey, under the aforesaid trade-mark designation.

20 In each formulation the base stock is prepared by milling together all the ingredients on standard rubber rolls until a homogeneous mixture is obtained. If it is desired to make only a small batch of the adhesive, the ingredients with the exception of the resin are first milled together on standard rubber rolls and the resin then added and blended into the mass in a Banbury mixer. The resulting blend of materials is then dissolved 25 in a suitable solvent such as methyl ethyl ketone, methyl isobutyl ketone, benzene and trichloroethylene, or the like in sufficient amount to produce an adhesive solution of the desired consistency. For example, in preparing an adhesive 30 solution from one of the base stock formulations above set forth the following proportions are found to provide adhesives of suitable consistency:

|                     | Per cent |
|---------------------|----------|
| 40 Base stock       | 30       |
| Methyl ethyl ketone | 70       |

35 There are a number of commercial adhesive products of the above blended rubber-resin type which I have found available on the market and which are suitable for use in carrying out the present invention. These commercial adhesives are basically a resin-modified rubber base stock, including various conventional modifying agents such as vulcanizers, antioxidants, accelerators and the like, dissolved or suspended in a vehicle or solvent such as methyl ethyl ketone, methyl isobutyl ketone, benzene or trichloroethylene, or other comparable solvent. Among the commercially available adhesives which I have found can be used satisfactorily for the production of my scouring pads are the following:

40 Du Pont No. 4665 adhesive, made and sold by E. I. du Pont de Nemours & Company of Wilmington, Delaware, and which is a butadiene-acrylonitrile copolymer blended with a phenol aldehyde resinous condensation product in the proportion of about 70 parts of the said copolymer to 30 parts of the phenolic resin dissolved in a suitable solvent.

45 Du Pont No. 4678 adhesive, made and sold by E. I. du Pont de Nemours & Company of Wilmington, Delaware, and which is also satisfactory is basically similar in composition and general properties to Du Pont No. 4665 adhesive.

50 "Pli-O-Bond" adhesive, made and sold by the U. S. Plywood Company, is a resin-modified butadiene-acrylic nitrile copolymer rubber dissolved in about 20% of methyl ethyl ketone.

55 The term "rubber" as used herein in the speci-

fication or the claims as applied to the rubber constituent of the adhesive used for securing the abrasive particles to the foam rubber backing is intended to include not only natural rubber but also include the various synthetic rubbers or elastomers available on the market such as butadiene-acrylonitrile copolymers, butadiene-styrene copolymers, polychloroprene and other types of synthetic rubber materials.

The foam rubber or latex foam which constitutes the backing or base layer of the scouring articles of the present invention is prepared directly from the milky latex of the rubber tree or from one of the synthetic latices compounded with the desired vulcanizing agent and other ingredients commonly used in the art. The foam rubber is usually made commercially by one of two processes,

- (a) The hydrogen peroxide frothing process, or
- (b) The whipping process.

Such foam rubbers or latex foam materials are to be distinguished from either chemically blown sponge rubbers or expanded rubbers which are considerably different. By contrast, chemically blown sponge rubber is made from solid slab rubber which is compounded with a blowing agent and the resulting compound baked like a cake. Upon heating, the blowing agent, for example an azo compound, decomposes to form a gas which causes the rubber to expand and fill the mold. If the extra gas is permitted to escape thereby causing the cells to break, a product having interconnected cells is produced. If an excess of blowing agent is not employed a closed cell, chemically blown sponge rubber is produced. Expanded sponge rubber is made by externally gassing solid slab rubber with nitrogen or other gas to yield a closed cell product. The various chemically blown sponge rubbers or expanded sponge rubbers, both of which are made by processing rubber masses in solid form, have been found unsatisfactory for the fabrication of scouring devices of the herein described type. Therefore, when reference is made to a foam rubber in the specification or claims it is intended to exclude from that term the various chemically blown or expanded sponge rubbers.

Where reference is made herein to the use of foam rubber as the backing material it is intended to include not only foam rubber made from a natural rubber latex but to also include foam rubber materials composed of or containing the various synthetic rubber latices in foamed condition such as the foamed latices of polychlo-

roprene, butadiene-acrylonitrile copolymers, butadiene-styrene copolymers and other types of synthetic rubbers or elastomers either alone or blended in various proportions with one another or with a natural rubber latex.

Having described the invention, it is desired to claim:

1. A scouring implement comprising a foam rubber backing and a single layer of abrasive granules substantially one grit size in thickness adhesively secured thereto by means of a water insoluble adhesive having permanent flexibility and elongation, said adhesive comprising a blend of rubber and thermosetting resin, said foam rubber backing being of sufficient thickness to impart compressibility and handling strength to the article.
2. A scouring implement comprising a foam rubber backing of sufficient thickness to impart compressibility and handling strength to the article and a single layer of abrasive granules substantially one grit size in thickness adhesively secured thereto by means of a thermosetting resin-modified rubber base adhesive.
3. A scouring implement comprising a foam rubber backing of sufficient thickness to impart compressibility and handling strength to the article and a single layer of abrasive granules substantially one grit size in thickness adhesively secured thereto by means of a water-insoluble adhesive comprising a blend of rubber and a phenol aldehyde resinous condensation product.
4. A scouring implement comprising a base layer of foam rubber from  $\frac{3}{8}$ " to 1" in thickness, a superposed layer of thermosetting resin-modified rubber base adhesive adhered thereto, and a single layer of particulate abrasive material substantially one grit size in thickness embedded in said adhesive layer and secured to the base layer thereby, said adhesive and base layers being permanently flexible, elastic and conformable to substantially the same degree and resistant to the action of hot water of the average temperature of dishwasher, and to the soaps, detergents, oils, fats, greases, solvents and chemicals found therein.

DON L. EASTMAN.

References Cited in the file of this patent  
UNITED STATES PATENTS

| Number    | Name            | Date          |
|-----------|-----------------|---------------|
| 60,264    | Sawyer          | Dec. 4, 1866  |
| 2,001,911 | Wooddell et al. | May 21, 1935  |
| 2,236,597 | Hatch           | Apr. 1, 1941  |
| 2,339,547 | Carter          | Jan. 18, 1944 |